



US005935694A

# United States Patent [19]

Olmstead et al.

[11] Patent Number: 5,935,694

[45] Date of Patent: Aug. 10, 1999

[54] FLUORESCENT SECURITY THERMAL TRANSFER PRINTING RIBBON

[75] Inventors: **Michael W. Olmstead**, Centerville; **Joseph D. Roth**; **Richard D. Puckett**, both of Miamisburg, all of Ohio[73] Assignee: **NCR Corporation**, Dayton, Ohio

[21] Appl. No.: 08/895,338

[22] Filed: Jul. 16, 1997

## Related U.S. Application Data

[60] Continuation of application No. 08/598,870, Feb. 9, 1996, abandoned, which is a division of application No. 08/092, 296, Jul. 15, 1993, Pat. No. 5,516,590.

[51] Int. Cl.<sup>6</sup> ..... B41M 5/26

[52] U.S. Cl. ..... 428/212; 428/195; 428/201; 428/484; 428/488.4; 428/690; 428/913; 428/914

[58] Field of Search ..... 428/195, 201, 428/690, 202, 204, 212, 484, 488.4, 913, 914

[56]

## References Cited

### U.S. PATENT DOCUMENTS

|           |         |                           |
|-----------|---------|---------------------------|
| 4,180,204 | 12/1979 | Koenig et al. ....        |
| 4,515,849 | 5/1985  | Keino et al. .... 428/204 |
| 5,568,177 | 10/1996 | Talvalkar et al. ....     |

Primary Examiner—Pamela R. Schwartz  
Attorney, Agent, or Firm—Craig E. Miller

[57]

## ABSTRACT

Fluorescent security thermal transfer printing ribbons consisting of an elongated backing element having a printing media adhered to one side thereof. The printing media is capable of being transferred to paper, or some other print receiving medium, by conventional thermal transfer printing equipment. The thermally transferred printing media includes an interspersed distribution of fluorescent pigments, resulting in printed security characters and images which are transparent or invisible under broad spectrum light, but which fluoresce, and become visible, when exposed to black light.

8 Claims, 4 Drawing Sheets



**FIG. 1****FIG. 2****FIG. 3**

**FIG. 4****FIG. 5****FIG. 6**

**FIG. 7****FIG. 8****FIG. 9**

**FIG. 10****FIG. 11**

## FLUORESCENT SECURITY THERMAL TRANSFER PRINTING RIBBON

This is a continuation of application(s) Ser. No. 08/598, 870 filed on Feb. 9, 1996, now abandoned which is a Division, of application Ser. No. 08/092,296, filed Jul. 15, 1993 now U.S. Pat. No. 5,516,590.

### BACKGROUND AND SUMMARY OF THE INVENTION

The present invention relates generally to new and novel improvements in fluorescent security printing ribbons. More particularly, the present invention relates to thermal transfer printing ribbons capable of printing security characters and indicia in conjunction with product identification bar codes and other visible printing, such that the security characters and indicia are invisible under broad spectrum light, but fluoresce, and become visible, when exposed to black light.

One prevalent problem in the retail industry is how to verify that merchandise sold to a customer was sold by a particular store. Although the name of the store could be visibly printed on the product's packaging, or directly on the product, doing so is sometimes undesirable to consumers who, for example, may want to give the purchased products to others as gifts, or may want to use the items without visible printing. In addition, if the store name is visible, it is readily apparent and could be fraudulently reproduced by unscrupulous individuals.

Accordingly, an object of the present invention is the provision of printing ribbons capable of printing security characters and indicia incorporated into, for example, product identification bar codes or other visible printing, such that the security characters and indicia are invisible under broad spectrum light, but fluoresce, and become visible, when exposed to black light.

Another object of the present invention is the provision of printing ribbons capable of printing security characters and indicia which are transparent, and thus invisible under broad spectrum light, but which fluoresce, and become visible, when exposed to black light.

A further object of the present invention is the provision of thermal transfer printing ribbons capable of printing fluorescent security characters and indicia using conventional thermal printing equipment.

Yet another object of the present invention is the provision of thermal transfer printing ribbons capable of printing product identification bar codes and other visible images under control of a thermal transfer print head and security characters and indicia controlled, at least in part, by predetermined spot coated patterns or configurations present on the thermal transfer printing ribbons prior to the printing operation.

These and other objects of the present invention are attained by the provision of printing ribbons consisting of elongated backing elements with printing media adhered to one side thereof. The printing media is preferably capable of being transferred to paper, or some other print receiving media, by conventional thermal transfer printing equipment. In one preferred embodiment, the thermally transferred printing media includes a uniform interspersed distribution of fluorescent pigments, resulting in printed security characters and images which are transparent, and thus invisible, under broad spectrum light, but which fluoresce, and become visible, when exposed to black light. In a second preferred embodiment, the thermally transferred printing media includes a uniform interspersed distribution of visible

black or colored pigments, as well as fluorescent pigments, resulting in printed product identification bar codes or other visible printed images which are visible under broad spectrum light, as well as printed security characters and indicia which are transparent, and thus invisible, under broad spectrum light, but which fluoresce, and become visible, when exposed to black light. If desired, the visible printed images or patterns can be made in one configuration, for example, conventional product identification bar codes, controlled by the thermal print head and the fluorescent security characters and indicia can be made in a different configuration, for example, the name of a particular store, or the store's logo, controlled, at least in part, by predetermined spot coated patterns or configurations present on the thermal printing ribbons prior to the printing operation. Thus, printing ribbons in accordance with this invention can be used to print visibly transparent printing, black printing, or other color printing as viewed under broad spectrum light, and independent fluorescent security characters and indicia which are invisible under broad spectrum light, but which fluoresce, and become visible, when exposed to black light.

Other objects, advantages and novel features of the present invention will become apparent in the following detailed description of the invention when considered in conjunction with the accompanying drawings.

### BRIEF DESCRIPTION OF THE DRAWINGS

FIG. 1 is a cross-sectional side view of a first preferred embodiment of a fluorescent security thermal transfer printing ribbon in accordance with the present invention having a single printing media layer with a uniform interspersed distribution of visible black or colored pigments and fluorescent pigments.

FIG. 2 is a cross-sectional side view of a second preferred embodiment of a fluorescent security thermal transfer printing ribbon in accordance with the present invention having a single printing media layer with a uniform interspersed distribution of fluorescent pigments.

FIG. 3 is a cross-sectional side view of a third preferred embodiment of a fluorescent security thermal transfer printing ribbon in accordance with the present invention having a first printing media layer with a uniform interspersed distribution of black or colored pigments and a second printing media layer with a uniform interspersed distribution of fluorescent pigments.

FIG. 4 is a cross-sectional side view of a fourth preferred embodiment of a fluorescent security thermal transfer printing ribbon in accordance with the present invention having a first printing media layer with a predetermined spot printed configuration of fluorescent pigment and a second printing media layer with a uniform interspersed distribution of black or colored pigments.

FIG. 5 is a top view of the fluorescent security thermal transfer printing ribbon shown in FIG. 4 showing the spot printed configuration of the first printing media layer adhered to the backing element without the second printing media layer.

FIG. 6 is a top view of a thermally transferred product identification bar code as printed on paper or some other print receiving medium using the fluorescent security thermal transfer printing ribbon shown in FIG. 4, as the product identification bar code would visibly appear under broad spectrum light.

FIG. 7 is a top view of a thermally transferred product identification bar code as printed on paper or some other print receiving medium using the fluorescent security ther-

mal transfer printing ribbon shown in FIG. 4, as the product identification bar code would visibly appear when exposed to black light.

FIG. 8 is a cross-sectional side view of a fifth preferred embodiment of a fluorescent security thermal transfer printing ribbon in accordance with the present invention having a first printing media layer with a uniform interspersed distribution of black or colored pigments, a second printing media layer with a predetermined spot printed configuration of fluorescent pigments, and a third printing media layer with a predetermined spot printed configuration of fluorescent pigments.

FIG. 9 is a top view of the fluorescent security thermal transfer printing ribbon shown in FIG. 8 showing the spot printed configuration of the second and third printing media layers adhered to the backing element without the first printing media layer.

FIG. 10 is a top view of a thermally transferred product identification bar code as printed on paper or some other print receiving medium using the fluorescent security thermal transfer printing ribbon shown in FIG. 8, as the product identification bar code visibly appear under broad spectrum light.

FIG. 11 is a top view of a thermally transferred product identification bar code as printed on paper or some other print receiving medium using the fluorescent security thermal transfer printing ribbon shown in FIG. 8, as the product identification bar code would visibly appear when exposed to black light.

#### DETAILED DESCRIPTION OF THE DRAWINGS

Referring now to the drawings, in which like-referenced characters indicate corresponding elements throughout the several views, attention is first drawn to FIG. 1 which illustrates a first preferred embodiment of a fluorescent security thermal transfer printing ribbon in accordance with the present invention, generally identified by reference numeral 10. Fluorescent security thermal transfer printing ribbon 10 consists of a single printing media layer 12 which is adhered to one side of elongated backing element 14. Backing element 14 is preferably a long narrow strip of a flexible polymeric material, such as Mylar, available from E. I. Dupont de Nemours & Co., Inc. in Wilmington, Del. Backing element 14 should be compatible with printing media layer 12, and preferably has sufficient tensile strength to resist tearing, while being sufficiently flexible to be wound around a spool or reel.

Printing media layer 12 preferably includes a uniform interspersed distribution of visible black or colored pigments 16 and fluorescent pigments 18 in binding substrate 20. Visible black or colored pigments 16 most preferably include carbon black pigments, but could also include visible green, brown, blue and other colored pigments. Visible black or colored pigments 16 allow the printed image to appear visibly black or colored, as desired, under broad spectrum light. Fluorescent pigments 18 are inactive under broad spectrum light, but fluoresce, and become visible, when exposed to black light.

Binding substrate 20 retains the uniform interspersed distribution of black or colored pigments 16 and fluorescent pigments 18 against backing element 14 prior to the printing operation. In addition, binding substrate 20 retains the uniform interspersed distribution of black or colored pigments 16 and fluorescent pigments 18 once printing media layer 12 is transferred onto paper or some other print receiving medium.

A preferred formulation for the first preferred embodiment of fluorescent security thermal transfer printing ribbon 10 shown in FIG. 1 is given below:

| Ingredient                 | % Dry | % Dry Range | Grams Dry | Grams Wet |
|----------------------------|-------|-------------|-----------|-----------|
| Mineral Spirits            | —     | —           | —         | 400.0     |
| Copolymer Resin            | 5.0   | 2-20%       | 5.0       | 5.0       |
| Thermoplastic Resin        | 10.0  | 5-25%       | 10.0      | 10.0      |
| Rice Bran Wax              | 65.0  | 45-75%      | 65.0      | 65.0      |
| Carbon Black Pigment       | 10.0  | 5-15%       | 10.0      | 10.0      |
| Ultraviolet Yellow Pigment | 10.0  | 5-15%       | 10.0      | 10.0      |
| Total                      | 100.0 |             | 100.0     | 500.0     |

In the above preferred formulation of fluorescent security thermal transfer printing ribbon 10, the copolymer resin used is marketed as "Lotryl 15MA03 Copolymer Resin" by Elf Atochem in Paris, France; the thermoplastic resin used is marketed as "Stereon 840-A Thermoplastic Resin" by Firestone Tire & Rubber Co. in Akron, Ohio; the rice bran wax used is marketed as "Rice Bran Wax" by Frank B. Ross Co., Inc. in Jersey City, N.J.; the carbon black pigment used is marketed as "Conductex SC Pigment" by Columbia Chemical in Atlanta, Ga.; the ultraviolet yellow pigment used is marketed as "UV Yellow Pigment" by Stroblite Co., Inc. in New York City, N.Y.; and the backing element used is marketed as "14.5 micron Polyester Film" by E. I. Dupont de Nemours & Co., Incorporated in Wilmington, Del.

To fabricate fluorescent security thermal transfer printing ribbon 10, a wax emulsion of mineral spirits, copolymer resin, thermoplastic resin and rice bran wax is made by mixing these ingredients together and heating the mixture to 190° F. for thirty minutes. Next, the carbon black pigment and ultraviolet yellow pigment are added and the resultant mixture is ground in an attritor for approximately ninety minutes. This mixture is then coated at 140-150° F. onto the backing element at a dry coat weight of 3.1+/-0.5 grams per square meter to form finished fluorescent security thermal transfer printing ribbon 10.

Referring now to FIG. 2, a second preferred embodiment of a fluorescent security thermal transfer printing ribbon in accordance with the present invention, generally identified by reference numeral 30, is shown. Fluorescent security thermal transfer printing ribbon 30 consists of a single printing media layer 32 which is adhered to one side of elongated backing element 34. As in the case of fluorescent security thermal transfer printing ribbon 10 shown in FIG. 1, backing element 34 is preferably a long narrow strip of a flexible polymeric material, such as Mylar, available from E. I. Dupont de Nemours & Co., Inc. in Wilmington, Del. Backing element 34 should be compatible with printing media layer 32, and preferably has sufficient tensile strength to resist tearing, while being sufficiently flexible to be wound around a spool or reel.

Printing media layer 32 preferably includes a uniform interspersed distribution of fluorescent pigments 38 in binding substrate 40. Fluorescent pigments 38 are inactive under broad spectrum light, but fluoresce, and become visible, when exposed to black light. Thus, images printed using fluorescent security thermal transfer printing ribbon 30 are transparent or invisible under broad spectrum light, but become visible when exposed to black light.

Binding substrate 40 retains the uniform interspersed distribution of fluorescent pigments 38 against backing

element **34** prior to the printing operation. In addition, binding substrate **40** retains the uniform interspersed distribution of fluorescent pigments **38** once printing media layer **32** is transferred onto paper or some other print receiving medium.

A preferred formulation for the second preferred embodiment of fluorescent security thermal transfer printing ribbon **30** shown in FIG. 2 is given below:

| Ingredient                 | % Dry | % Dry Range | Grams Dry | Grams Wet |
|----------------------------|-------|-------------|-----------|-----------|
| Mineral Spirits            | —     | —           | —         | 400.0     |
| Copolymer Resin            | 5.0   | 2-20%       | 5.0       | 5.0       |
| Thermoplastic Resin        | 10.0  | 5-25%       | 10.0      | 10.0      |
| Rice Bran Wax              | 65.0  | 45-75%      | 65.0      | 65.0      |
| Ultraviolet Yellow Pigment | 20.0  | 15-25%      | 20.0      | 20.0      |
| Total                      | 100.0 |             | 100.0     | 500.0     |

In the above preferred formulation of fluorescent security thermal transfer printing ribbon **30**, the copolymer resin used is marketed as "Lotryl 15MA03 Copolymer Resin" by Elf Atochem in Paris, France; the thermoplastic resin used is marketed as "Stereon 840-A Thermoplastic Resin" by Firestone Tire & Rubber Co. in Akron, Ohio; the rice bran wax used is marketed as "Rice Bran Wax" by Frank B. Ross Co., Inc. in Jersey City, N.J.; the ultraviolet yellow pigment used is marketed as "UV Yellow Pigment" by Stroblite Co., Inc. in New York City, N.Y.; and the backing element used is marketed as "4.5 micron Polyester Film" by E. I. Dupont de Nemours & Co., Incorporated in Wilmington, Del.

To fabricate fluorescent security thermal transfer printing ribbon **30**, a wax emulsion of mineral spirits, copolymer resin, thermoplastic resin and rice bran wax is made by mixing these ingredients together and heating the mixture to 190° F. for thirty minutes. Next, the ultraviolet yellow pigment is added and the resultant mixture is ground in an attritor for approximately ninety minutes. This mixture is then coated at 140-150° F. onto the backing element at a dry coat weight of 3.1+/-0.5 grams per square meter to form finished fluorescent security thermal transfer printing ribbon **30**.

Referring now to FIG. 3, a third preferred embodiment of a fluorescent security thermal transfer printing ribbon in accordance with the present invention, generally indicated by reference numeral **50**, is shown. Fluorescent security thermal transfer printing ribbon **50** consists of first printing media layer **52** which is adhered to one side of elongated backing element **54**, and second printing media layer **62** which is adhered to the surface of first printing media layer **52** distal from backing element **54**. As in the case of fluorescent security thermal transfer printing ribbon **10** shown in FIG. 1, backing element **54** is preferably a long narrow strip of a flexible polymeric material, such as Mylar, available from E. I. Dupont de Nemours & Co., Inc. in Wilmington, Del. Backing element **54** should be compatible with first printing media layer **52**, and preferably has sufficient tensile strength to resist tearing, while being sufficiently flexible to be wound around a spool or reel.

First printing media layer **52** preferably includes a uniform interspersed distribution of fluorescent pigments **58** in binding substrate **60**. Second printing media layer **62** preferably includes a uniform interspersed distribution of visible black or colored pigments **56** in binding substrate **64**. Thus, images printed using fluorescent security thermal transfer

printing ribbon **50** consist of a bottom layer of second printing media layer **62** with a uniform interspersed distribution of visible black or colored pigments **56** in binding substrate **64** and a top layer of first printing media layer **52** with a uniform interspersed distribution of fluorescent pigments **58** in binding substrate **60**. Since fluorescent pigments **58** are transparent, and thus invisible under broad spectrum light, visible black or colored pigments **56** allow the printed images to appear visibly black or colored, as desired, under broad spectrum light. However, fluorescent pigments **58** fluoresce, and become visible, when exposed to black light.

Binding substrate **60** retains the uniform interspersed distribution of fluorescent pigments **58** against backing element **54** prior to the printing operation. Similarly, binding substrate **64** retains the uniform interspersed distribution of visible black or colored pigments **56** prior to the printing operation. In addition, binding substrate **60** retains the uniform distribution of fluorescent pigments **58** and binding substrate **64** retains the uniform interspersed distribution of visible black or colored pigments **56** once second printing media layer **62** and first printing media layer **52** are transferred onto paper or some other print receiving medium.

Referring now to FIGS. 4 and 5, a fourth preferred embodiment of a fluorescent security thermal transfer printing ribbon in accordance with the present invention, generally indicated by reference numeral **70**, is shown. Fluorescent security thermal transfer printing ribbon **70** consists of first spot coated printing media layer **72** which is adhered to one side of elongated backing element **74**, and second printing media layer **82** which is adhered to the surface of first spot coated printing media layer **72** distal from backing element **74** and to portions of backing element **74** not covered by first spot coated printing media layer **72**. As in the case of fluorescent security thermal transfer printing ribbon **10** shown in FIG. 1, backing element **74** is preferably a long narrow strip of a flexible polymeric material, such as Mylar, available from E. I. Dupont de Nemours & Co., Inc. in Wilmington, Del. Backing element **74** should be compatible with first spot coated printing media layer **72** and second printing media layer **82**, and preferably has sufficient tensile strength to resist tearing, while being sufficiently flexible to be wound around a spool or reel.

First spot coated printing media layer **72** preferably includes a uniform interspersed distribution of fluorescent pigments **78** in binding substrate **80** spot coated in any desired pattern or configuration on backing element **74**. For example, first spot coated printing media layer **72** could be spot coated in a pattern or configuration identifying a particular store's name, logo or some other desired identifiable configuration, as represented by repeating pattern **86** of ABC's shown in FIG. 5. Second printing media layer **82** preferably includes a uniform interspersed distribution of visible black or colored pigments **76** in binding substrate **84**. Images printed using fluorescent security thermal transfer printing ribbon **70** consist of a bottom layer of second printing media layer **82** with a uniform interspersed distribution of visible black or colored pigments **76** in binding substrate **84** and a top layer of first spot coated printing media layer **72** with the spot coated pattern or configuration of uniform interspersed distribution of fluorescent pigments **78** in binding substrate **80**. Since fluorescent pigments **78** are transparent, and thus invisible under broad spectrum light, visible black or colored pigments **76** allow the printed images to appear visibly black or colored, as desired, under broad spectrum light as shown in FIG. 6. Fluorescent pigments **78** present in repeating pattern **86** fluoresce, and become visible, when exposed to black light as shown in FIG. 7.

Binding substrate 80 retains the spot coated uniform interspersed distribution of fluorescent pigments 78 against backing element 74 prior to the printing operation. Similarly, binding substrate 84 retains the uniform interspersed distribution of visible black or colored pigments 76 prior to the printing operation. In addition, binding substrate 80 retains the spot coated uniform interspersed distribution of fluorescent pigments 78 and binding substrate 84 retains the uniform interspersed distribution of visible black or colored pigments 76 once second printing media layer 82 and first spot coated printing media layer 72 are transferred onto paper or some other printing medium.

Referring now to FIGS. 8 and 9, a fifth preferred embodiment of a fluorescent security thermal transfer printing ribbon in accordance with the present invention, generally indicated by reference numeral 90, is shown. Fluorescent security thermal transfer printing ribbon 90 consists of first spot coated printing media layer 92 which is adhered to one side of elongated backing element 94, second spot coated printing media layer 102 which is adhered to the same side of backing element 94, and third printing media layer 108 which is adhered to the surfaces of first spot coated printing media layer 92 and second spot coated printing media 102 distal from backing element 94 and to portions of backing element 94 not covered by first spot coated printing media layer 92 and second spot coated printing media layer 102. As in the case of fluorescent security thermal transfer printing ribbon 10 shown in FIG. 1, backing element 94 is preferably a long narrow strip of a flexible polymeric material, such as Mylar, available from E. I. Dupont de Nemours & Co., Inc. in Wilmington, Del. Backing element 94 should be compatible with first spot coated printing media layer 92, second spot coated printing media layer 102 and third spot coated printing media layer 108, and preferably has sufficient tensile strength to resist tearing, while being sufficiently flexible to be wound around a spool or reel.

First spot coated printing media layer 92 preferably includes a uniform interspersed distribution of fluorescent pigments 98 in binding substrate 100 spot coated in any desired pattern or configuration on backing element 94. Similarly, second spot coated printing media layer 102 preferably includes a uniform interspersed distribution of fluorescent pigments 110 in binding substrate 104 spot coated in any desired pattern or configuration on backing element 94. For example, first spot coated printing media layer 92 could be spot coated in a first pattern or configuration as represented by repeating pattern 106 of ABC's shown in FIG. 9, identifying, for example, a particular store's name, and second spot coated printing media layer 102 could be spot coated in a second pattern or configuration as represented by repeating pattern 112 of XYZ's shown in FIG. 9, identifying, for example, a particular store's logo or some other identifiable configuration. If desired, second spot coated printing media layer 102 could be allowed to overlap first spot coated printing media layer 92 in a predetermined manner. Third printing media layer 108 preferably includes a uniform interspersed distribution of visible black or colored pigments 96 in binding substrate 114.

Images printed using fluorescent security thermal transfer printing ribbon 90 consist of a bottom layer of third printing media layer 108 with a uniform interspersed distribution of visible black or colored pigments 96 in binding substrate 114 and a top layer of first spot coated printing media layer 92 with the spot coated pattern or configuration of uniform interspersed distribution of fluorescent pigments 98 in binding substrate 100 and second spot coated printing media layer 102 with the spot coated pattern or configuration of

uniform interspersed distribution of fluorescent pigments 110 in binding substrate 104. Since fluorescent pigments 98 and 110 are transparent, and thus invisible under broad spectrum light, visible black or colored pigments 96 allow the printed images to appear visibly black or colored, as desired, under broad spectrum light as shown in FIG. 10. Fluorescent pigments 98 present in repeating pattern 106 and fluorescent pigments 110 present in repeating pattern 112 fluoresce, and become visible, when exposed to black light as shown in FIG. 11. If desired, fluorescent pigments 98 could be a different color or concentration than fluorescent pigments 110 so repeating pattern 106 of fluorescent pigments 98 would appear as a different color or intensity, and thus would be visually distinguishable from repeating pattern 112 of fluorescent pigments 110, when exposed to black light.

Binding substrate 100 retains the spot coated uniform interspersed distribution of fluorescent pigments 98 and binding substrate 104 retains the spot coated uniform interspersed distribution of fluorescent pigments 110 against backing element 94 prior to the printing operation. Similarly, binding substrate 114 retains the uniform interspersed distribution of visible black or colored pigments 96 prior to the printing operation. In addition, binding substrate 100 retains the spot coated uniform interspersed distribution of fluorescent pigments 98, binding substrate 104 retains the spot coated uniform interspersed distribution of fluorescent pigments 110, and binding substrate 114 retains the uniform interspersed distribution of visible black or colored pigments 96 once third printing media layer 108, second spot coated printing media layer 102, and first spot coated printing media layer 92 are transferred onto paper or some other print receiving medium.

Although the present invention has been described above in detail, the same is by way of illustration and example only and is not to be taken as a limitation on the present invention. For example, although the use of two spot coated printing media layers has been described herein, the use of three, or even more, such spot coated media layers could be readily accomplished utilizing the teachings of present invention. Accordingly, the scope and content of the present invention are to be defined only by the terms of the appended claims.

#### What is claimed is:

1. A fluorescent security thermal transfer printing ribbon for printing a printed image having security characters or indicia, said fluorescent security thermal transfer printing ribbon comprising:
  - a backing element having a top surface;
  - a first printing media layer adhered to said top surface of said backing element, said first printing media layer having an interspersed distribution of fluorescent pigments and a top surface, said fluorescent pigments are transparent under broad spectrum light; and
  - a second printing media layer adhered to said top surface of said first printing media layer so that substantially the entire top surface of said backing element is covered by said second printing media layer, said second printing media layer having an interspersed distribution of visible black or colored pigments;
 wherein said first printing media layer forms the printed image security characters or indicia and said second printing media layer forms the printed image visible under broad spectrum light.
2. The fluorescent security thermal transfer printing ribbon in accordance with claim 1, wherein said first printing media layer is spot coated on said top surface of said backing

element in a predetermined pattern to cover a portion, but not all, of said top surface of said backing element.

3. The fluorescent security thermal transfer printing ribbon in accordance with claim 2, wherein:

10  
said fluorescent security thermal transfer printing ribbon includes a third spot coated printing media layer adhered to said top surface of said backing element, said third spot coated printing media layer having an interspersed distribution of fluorescent pigments and a top surface; and

said second printing media layer is adhered to said top surface of said first printing media layer and said top surface of said third spot coated printing media layer.

4. The fluorescent security thermal transfer printing ribbon in accordance with claim 3, wherein said fluorescent pigments in said first printing media layer are of a different color than said fluorescent pigments in said third printing media layer. 15

5. The fluorescent security thermal transfer printing ribbon in accordance with claim 3, wherein said fluorescent pigments in said first printing media layer are of a different concentration than said fluorescent pigments in said third printing media layer. 20

6. The fluorescent security thermal transfer printing ribbon in accordance with claim 3, wherein said third printing media layer overlaps a portion of said first printing media layer. 25

7. The fluorescent security thermal transfer printing ribbon in accordance with claim 2, wherein said predetermined pattern is a repeating pattern.

8. A fluorescent security thermal transfer printing ribbon for printing a printed image having security characters or indicia, said fluorescent security thermal transfer printing ribbon comprising:

a backing element having a top surface;  
a first printing media layer adhered to said top surface of said backing element, said first printing media layer having an interspersed distribution of fluorescent pigments, a top surface and being spot coated on said top surface of said backing element in a predetermined pattern to cover a portion, but not all, of said top surface of said backing element, said fluorescent pigments are transparent under broad spectrum light; and

a second printing media layer adhered to said top surface of said first printing media layer and to said backing element on portions not covered by said first printing media layer, said second printing media layer having an interspersed distribution of visible black or colored pigments;

wherein said first printing media layer forms the printed image security characters or indicia and said second printing media layer forms the printed image visible under broad spectrum light.

\* \* \* \* \*